

Jan. 28, 1969

S. HARTMAN ET AL  
VISCOELASTIC SOUND-BLOCKING MATERIAL WITH  
FILLER OF HIGH DENSITY PARTICLES

Filed May 12, 1965

3,424,270

Sheet 1 of 3

FIGURE 1



FIGURE 2



**INVENTORS**

FRANCIS F. SULLIVAN

BY Seymour Hartman

*James J. Heilman*  
ATTORNEY

Jan. 28, 1969

S. HARTMAN ET AL  
VISCOELASTIC SOUND-BLOCKING MATERIAL WITH  
FILLER OF HIGH DENSITY PARTICLES

3,424,270

Filed May 12, 1965

Sheet 2 of 3

FIG. 3



INVENTORS  
FRANCIS F. SULLIVAN  
BY Seymour Hartman

*James M. Heilman*  
ATTORNEY

Jan. 28, 1969

S. HARTMAN ET AL

3,424,270

VISCOELASTIC SOUND-BLOCKING MATERIAL WITH  
FILLER OF HIGH DENSITY PARTICLES

Filed May 12, 1965

Sheet 3 of 3

FIG. 4.



FIG. 5.



INVENTORS  
FRANCIS F. SULLIVAN  
SEYMOUR HARTMAN

BY

*James D. Heilman*

ATTORNEY.

## 1

3,424,270

VISCOELASTIC SOUND-BLOCKING MATERIAL  
WITH FILLER OF HIGH DENSITY PARTICLES  
Seymour Hartman, Mahopac, N.Y., and Francis F. Sullivan, Santa Barbara, Calif., assignors to U.S. Plywood-Champion Paper Inc., a corporation of New York  
Continuation-in-part of abandoned application Ser. No. 317,204, Oct. 18, 1963. This application May 12, 1965, Ser. No. 455,247  
U.S. Cl. 181—33 10 Claims  
Int. Cl. G10k 11/04; E04b 1/99

The present invention is a continuation-in-part of applicants' copending application Ser. No. 317,204, filed October 18, 1963, now abandoned and is broadly concerned with a novel composition of matter which possesses the physical properties of mass and viscoelasticity and also with its method of manufacture. The invention is further concerned with the application of these materials or compositions possessing both mass and viscoelasticity for the preparation of high quality acoustical structural units as, for example, a panel, a wall, a ceiling, a floor, or any partition wherein it is desired that it possess high acoustical or a high sound transmission loss, and in X-ray and radiation shielding. Such a composition of matter which comprises mass in a viscoelastic matrix will also find use in the manufacturing of high quality stereo speaker enclosures; whereby proper response of either very low and very high frequencies can be achieved. This viscoelastic mass is incapable of resonating, no matter how strong the bass backwave is projected against it. Optimum results are achieved with the very low frequency range since all vibrations are damped. In particular, the composition of the present invention comprises a high density viscoelastic material which functions, when incorporated in an acoustical structural unit, to provide an exceptionally high acoustical sound barrier.

It is known in the art that sound or sound waves are blocked or attenuated by mass or weight of a structural element. Generally speaking, the greater the mass or weight per unit area of the structural element such as mass per square foot, the greater will be the sound transmission loss or the greater the sound attenuation on the other side of the element. On the other hand, it is also known in the acoustic art that the weight or mass is fully effective only if the panel is perfectly "limp." When the panel is limp and the sound waves strike the structural element, the resulting motion is localized and the sound spreads quite slowly. Thus, the acoustical efficiency with respect to attenuation of sound waves of any material depends not only on its weight per unit area, but also on its "bending stiffness." If a panel or structural element is too stiff or too rigid, it will actually lose much of its attenuation characteristics which it gains by having a relatively high mass per unit area. Thus, to attain an ideal system for acoustical barriers, it is necessary that the attenuation unit have both high weight or mass per unit area and also have bending stiffness (limpness). Limpness in the present application will be referred to as viscoelasticity.

The composition of the present invention of a high density and viscoelastic material is utilized to produce structural units having high acoustical attenuation or which produces a very high sound transmission loss. The composition of the present invention is obtained by utilizing a solid material as an inorganic filler. The preferred solid material comprises barium sulfate which has an overall specific gravity of about 4.5. The solid material such as the preferred barium sulfate is homogeneously dispersed in a viscoelastic binder.

Barium sulphate is particularly important because of its availability and cheapness. For example, while the cost of lead ranges from about 15 to 18 cents per pound, barium sulphate ranges from 1 to 2 cents per pound.

## 2

While barium sulphate is greatly preferred, other dense materials may be used providing they possess a specific gravity preferably above 4.0 or at the minimum above 3.0.

Compounds of elements which fall into this category possess one or more of the following anionic moieties, the sulfide, the oxide, the carbide, the iodide, the boride, the selenide, the chloride, the silicide, the telluride, the carbonate and/or the sulfate. One or more of the above mentioned anionic groups of the following elements (listed below), possess a density of 4 or more:

|    |           |            |
|----|-----------|------------|
| 10 | Vanadium  | Europium   |
|    | Tantalum  | Gallium    |
|    | Tellurium | Indium     |
|    | Thorium   | Iron       |
| 15 | Tin       | Lead       |
|    | Tungsten  | Magnesium  |
|    | Zinc      | Manganese  |
|    | Zirconium | Molybdenum |
|    | Aluminium | Neodymium  |
| 20 | Antimony  | Nickel     |
|    | Arsenic   | Niobium    |
|    | Barium    | Osmium     |
|    | Bismuth   | Palladium  |
|    | Calcium   | Platinum   |
| 25 | Cadmium   | Rhodium    |
|    | Cerium    | Silver     |
|    | Chromium  | Sodium     |
|    | Copper    | Strontium  |

30 Of the foregoing, preferred substances are lead sulfide, lead iodide, thorium boride, lead carbonate and strontium carbonate. Other good substances are iron carbonate and iron boride.

35 While relatively large particles of solid filler may be embedded throughout the mass of the binder as, for example, particles which pass through about 100 mesh screen, it is preferred that the particles utilized be relatively fine as, for example, a mass of particles wherein at least 90% pass through a 250 mesh screen, and preferably a mass of particles wherein at least 90% pass through a 325 mesh screen. When relatively fine particles are used, a very high quality acoustical panel is secured. This solid material added to the binder as mentioned should have specific gravity at least of 3.0 and preferably not less than about 4.0.

50 45 The viscoelastic binder components of the described sound blocking composition of the present invention may be any thermoplastic and/or modified flexible thermosetting resin which can be formulated with a high concentration by weight of barium sulfate, or other satisfactory substance as described, and others with similar specific gravities to yield an end viscoelastic material of high density. Materials or resins which are preferred are, for example, polyvinyl chloride, polyisobutylene, all natural and synthetic rubbers, polysulfides, flexible phenolics, polyurethanes (flexible), polyvinyl butyral, polyethylene-polyvinyl acetate copolymers, acrylonitrile rubbers, asphalt, tar, and combinations of the foregoing materials.

55 60 This high density and viscoelastic composition which is utilized for the production of acoustical structural units having a high degree of sound transmission loss is obtained by evenly and uniformly distributing the barium sulfate, or other high density material, or other similar materials with similar specific gravities within the viscoelastic binder, preferably under high shear. One technique or process for the manufacture of the composition of the present invention is to uniformly mix the barium sulfate in a viscoelastic binder under high shear by mixing in a unit as, for example, a Banbury Mill or on a "3-roll mill" or any other type of high shear mixing unit.

65 70 In general, it is preferred that the acoustical barium composition of the invention have a mass per square foot

in the range from about 0.5 lbs. to 20 lbs. per square foot, depending upon the sound transmission loss desired. A preferred range is from about 3 to 12 or 14 lbs./sq. ft. In general, the amount of barium sulfate, or other high specific gravity material, present in the sound blocking component is in the range from about 50 to 95%, preferably in the range of about 70 to 90% by weight as compared to from about 5 to 50% or 10 to 30% by weight of the viscoelastic binder or matrix. A very desirable concentration of barium sulfate is about 85% by weight.

After a homogeneous blend of the filler such as barium sulfate is secured in the viscoelastic binder, the blend or sound blocking composition is cured at a temperature in the range from about 150 to 350° F., preferably at about 275 to 330° F. for a time period in the range from about 15 minutes to 2 hours, preferably for a time period from about 1 to 1½ hours. It is to be understood that the temperature of curing as well as the time of curing is dependent upon the thickness of the composition desired as well as upon the binder used and also upon the weight per square foot.

It is preferred that the slabs be cured under pressure in the range from about 100 to 2000 lbs. per square inch. After curing of the high mass viscoelastic composition comprising barium sulfate in a binder, the material can then be used as a core material for the manufacture of structural units which possess high sound transmission losses.

The present invention may be more readily understood by reference to the drawings illustrating embodiments of the same.

FIGURE 1 illustrates a single core structural element.

FIGURE 2 illustrates a laminated core structure.

FIGURE 3 illustrates sound transmission loss of test specimens.

FIGURE 4 is a modified construction; and

FIGURE 5 is a further modified construction.

Referring specifically to FIGURE 1, the composition is employed as a core material 2 between two face panels 1 and 3 to produce an acoustical structural unit having a high sound transmission loss. Face panels 1 and 3 are of any material such as metal, asbestos, cement-asbestos, solid wood, wood veneer, hardboard, plywood, etc., which function as a front and back face of a structural unit, such as a door, a partition, a panel, a wall, a floor, or the like. The thickness of these panels may be of any desired thickness as, for example, from ¼" to 1" in thickness. Generally, it is preferred that if these panels are wood, they comprise about three plies. For example, the homogeneous blended slab 2, employed here as the core component, comprises the composition of a high percent by weight of barium sulfate uniformly distributed in a viscoelastic binder. The thickness of the core may vary appreciably depending upon other factors such as its use, the other dimensions, and the degree to which it is desired to cause sound transmission loss. Generally, the thickness of the core will be in the range from about ¼" to 3", preferably in the range from about ¼" to 1" for wall panels. Preferred overall thicknesses including the faces are from about ¾" to 2.5".

In order to further illustrate the invention, a number of operations were carried out in which high sound transmission loss panels were prepared employing the sound dampening or sound blocking compositions hereinbefore described. These operations are described in the following examples.

#### EXAMPLE 1

The following composition produced a high density viscoelastic material which, when fabricated into a core material as described, produced a panel having high sound transmission loss characteristics.

#### Parts by weight

|                          |     |
|--------------------------|-----|
| Polyvinyl chloride       | 400 |
| Plasticizer <sup>1</sup> | 410 |

|                           |      |
|---------------------------|------|
| Kenflex A <sup>2</sup>    | 200  |
| Celluflex 23 <sup>3</sup> | 20   |
| Barium sulfate            | 5200 |
| 6230                      |      |

|                                                                                                                                                                                                                                  |  |
|----------------------------------------------------------------------------------------------------------------------------------------------------------------------------------------------------------------------------------|--|
| 1 Tricresyl phosphate—170                                                                                                                                                                                                        |  |
| Diethyl phthalate—120                                                                                                                                                                                                            |  |
| Diiso-octyl phthalate—120                                                                                                                                                                                                        |  |
| 2 Synthetic polymer of aromatic hydrocarbons                                                                                                                                                                                     |  |
| (CH <sub>3</sub> ) <sub>2</sub> —C <sub>10</sub> H <sub>5</sub> —CH <sub>2</sub> —C <sub>10</sub> H <sub>4</sub> (CH <sub>3</sub> ) <sub>2</sub> CH <sub>2</sub> —C <sub>10</sub> H <sub>5</sub> (CH <sub>3</sub> ) <sub>2</sub> |  |

avg. mol. wt., 662; melting point, 160.

<sup>3</sup> Alkyl epoxy stearate (4.5% oxirane oxygen) (Celanese Chem. Co.).

The base plastisol was made up in a Hobart Mixer. One-half the amount of plasticizers was placed in the Hobart Mixer, and while being stirred the vinyl resin was added slowly. After homogeneous blending of the resin in the plasticizers, melted Kenflex A was added while being stirred. The inorganic barium sulfate was also added slowly while being stirred and the other half of the plasticizers was added as needed.

After admixing the above components the mass was milled two times on a three-roll mill to obtain a homogeneous mass. This material was then cured in slab forms at 327° F. for one hour to yield the viscoelastic dense sound blocking component employed as the core of a panel structure. Contact adhesives were coated on the two surfaces of this core structure as well as on two faces of the panels. When the contact cement was dried the high density viscoelastic core material was placed between the two outer face panels and run through a nip roll to make contact.

#### EXAMPLE 2

Another composition prepared as described is as follows:

|                                 | Parts by weight |
|---------------------------------|-----------------|
| 35 Powdered nitrile rubber      | 200             |
| Polyvinyl chloride              | 150             |
| Plasticizer                     | 200             |
| Stabilizer (vinyl) <sup>1</sup> | 5               |
| 40 Barium sulfate               | 1500            |
|                                 | 2055            |

<sup>1</sup> Barium cadmium stabilizer.

The resinous components were blended as in Example 1 in the plasticizers and milled on a three-roll mill. The milled mass was placed between two sheets of plywood and compressed to a thickness of 1" and held between the press at 300° F. for 15 minutes. If more viscoelasticity is desired, then addition of more plasticizer is required.

#### EXAMPLE 3

Another composition prepared as described is as follows:

|                        | Parts by weight |
|------------------------|-----------------|
| 55 Natural rubber      | 100             |
| Zinc oxide             | 5               |
| Stearic acid           | 2               |
| Amax <sup>1</sup>      | 1               |
| Methyl zimate          | 0.25            |
| Sulfur                 | 0.75            |
| 60 Reogen <sup>2</sup> | 5               |
| Barium sulfate         | 570             |
|                        | 686             |

<sup>1</sup> N-oxydiethylene benzothiazole-2-sulfenamide.

<sup>2</sup> Mixture of oil soluble sulfonic acid of high molecular weight with a paraffin oil.

The above components were milled on a Banbury Mill according to the usual methods employed in the rubber industry.

Slabs were then made and cured for about 30 minutes at 307° C. in the press under pressure ranging from 880 to 2000 lbs. or 200 to 800 p.s.i.

Also, variation in viscoelastic properties can be obtained in the foregoing example by (1) reducing the sulfur content, and (2) by employing plasticizers.

5  
EXAMPLE 4

Other slabs of the core composition described in Example 3 were prepared as follows: After milling on a Banbury Mill, two  $\frac{1}{8}$ " sheets of the above-formulated material was calendered into 4' x 8' x  $\frac{1}{8}$ " sheets. These two sheets were cured separately as described under similar conditions. Two other 4' x 8' x  $\frac{1}{4}$ " sheets were calendered from the same formulated stock and placed one on top of the other giving a 4' x 8' x  $\frac{1}{2}$ " uncured slab.

To this 4' x 8' x  $\frac{1}{2}$ " uncured slab was laminated on 10 the top and bottom using rubber contact cement, the two cured 4' x 8' x  $\frac{1}{8}$ ", thereby making up a laminated composition or structure consisting of a top 4' x 8' x  $\frac{1}{8}$ " cured high specific gravity viscoelastic material, followed by an intermediate 4' x 8' x  $\frac{1}{2}$ " uncured high specific gravity viscoelastic composition and finally a lower 4' x 8' x  $\frac{1}{8}$ " cured high specific gravity viscoelastic composition. This construction is preferred for some uses because of its exceedingly high and unobvious damping effects.

This laminated composition comprises the core used 20 in making up an acoustical panel secured by affixing two panels, such as, three-ply plywood, on the top and bottom using contact cement. The described acoustical panel is illustrated in FIGURE 2 wherein 10 and 11 are the two face panels of plywood or other material. The cured core laminated  $\frac{1}{8}$ " layers or sheets are shown as 12 and 13 while 14 and 15 show the double  $\frac{1}{4}$  inch sheets of the uncured composition. The resulting panel had a thickness of about  $1\frac{3}{4}$ ".

This panel manufactured as described was sent to 30 Riverbank Acoustical Laboratories located at Geneva, Ill., and tested for its acoustical properties; namely, its sound transmission loss.

The results of these tests<sup>1</sup> were as follows:

|                              |    |
|------------------------------|----|
| (A) Nine frequency average   | 42 |
| (B) Sound transmission class | 44 |

<sup>1</sup> These tests were conducted as described in their publication entitled "Special Report—Sound Transmission Class: An Explanation," 5th edition, dated June 15, 1962; and in their publication entitled "The Measurement of Airborne Sound Transmission Loss," dated May 1963.

A curve plotting the nine frequency results and sound transmission class is given in FIGURE 3.

The method used in making these measurements meets explicitly both the American Society for Testing and Materials Designation: E90-61T and the American Standard Recommended Practice: Z24.19-1957 for the measurement of airborne sound transmission loss.

The experimental panel,  $1\frac{1}{2}$ " thick by 44" wide by 84" high, was mounted in a frame made of 2 by 6" 50 lumber, using a P-gasket on one side and solid wood stops on the opposite side. The specimen consisted of a  $\frac{3}{8}$ " plywood on each side of a core containing 4 layers of a proprietary material. The frame was set into a 16" thick dense concrete filler wall of known transmission loss, which had been built in the source room opening. The specimen, less frame, weighed 341 lbs., an average of 13.3 lbs. per sq. ft. The transmission area, S, used in the computations was 25.6 sq. ft.

The sound transmission loss of a specimen (TL) is 60 the ratio, expressed in decibels, of the incident sound power on the source side of the specimen to the transmitted sound power on the receiving side when the sound fields on both sides of the specimen are diffused. The curve in the accompanying graph, FIG. 3, is the sound 65 transmission loss of the test specimen as derived from the measurement. The broken line is the sound transmission class contour. Sound transmission loss values are tabulated at eleven frequencies. The sound power transmitted by the filler wall was calculated and found to make no 70 significant change in the measured results as reported to the nearest decibel.

The nine-frequency arithmetic average, which excludes the values at 1400 and 2800 c.p.s., is given for comparison with previous data and for dealing with specifica- 75

tions still based on this index. A preferred criterion, based on actual partition requirements in typical architectural applications, is the sound transmission class.

A straight line can be drawn between the two check marks on the edges of the grid to locate the theoretical transmission loss of a limp mass with the same weight per sq. ft. as the specimen. This is given by the equation  $TL=20 \log W + 20 \log f - 33$ , where W is the weight in lb. per sq. ft. and F is the frequency in c.p.s.

In essence, the sound transmission loss measurements were made in accordance with applicable standards of the American Society for Testing and Materials, and the American Standards Association, Inc. identified as follows:

Tentative Recommended Practice for Laboratory Measurement of Airborne Sound Transmission Loss of Building Floors and Walls, ASTM designation: E90-61T.

American Standard Recommended Practice with the same title, Z24.19-1957.

Tentative method of Test for Sound Absorption of Acoustical Materials in Reverberation Rooms. ASTM designation: C423-60T.

American Standard Preferred Frequencies for Acoustical Measurements, S1.6-1960.

American Standard Acoustical Terminology, S1-1-1960.

It is to be understood that while a laminated component or panel such as described in Example 4 is very desirable, a component or panel can be manufactured solely from a totally cured viscoelastic mass and then coated with a paint, vinyl film or vinyl sheet, or wood veneer, etc.

Various other types of laminated products may be made, such as illustrated in FIG. 4 wherein the dense viscoelastic core is backed on one side with mineral fibers, acoustical plaster, cellulose fibers, particle board 30, etc. to which a thin facing of vinyl film or decorative wood veneer 31 is bonded. On the reverse side, there is laminated plaster-board, hardboard, plywood 32, etc.

Likewise, FIG. 5 illustrates different types of backing or facing materials such as absorbent fibrous material or acoustical plaster 33, and particle board or insulation board 34. Obviously, the core could be laminated with cured and uncured plies as illustrated in FIG. 2 if desired.

EXAMPLE 5

Another composition in accordance with the present invention is as follows:

|                           |     |
|---------------------------|-----|
| Vinyl resin <sup>1</sup>  | 50  |
| Hycar 1411 <sup>2</sup>   | 43  |
| Hycar 1312 <sup>3</sup>   | 100 |
| Paraplex G50 <sup>4</sup> | 45  |
| Stearic acid              | 1   |
| Zinc oxide                | 5   |
| Sulfur                    | 2   |
| Aluminum oxide (filler)   | 700 |
|                           | 946 |

<sup>1</sup> Exemplified by trademarks Geon of B. F. Goodrich, Marvinal of U.S. Rubber, and Opalon of Monsanto. A polyvinyl chloride resin (used for plastisol formulations). Specific viscosity 0.50-0.53; specific gravity, 1.4; particle size (micron 1-7).

<sup>2</sup> Trademark of B. F. Goodrich Chemical Company for their copolymer of butadiene and acrylonitrile of high acrylonitrile content. Specific gravity of 1.0. Average Mooney viscosity =115.

<sup>3</sup> Trademark of B. F. Goodrich Chemical Company for their copolymer of butadiene and acrylonitrile of medium-high acrylonitrile content. A liquid (100% solid) with a specific gravity=0.98.

<sup>4</sup> A trademark of Rohm & Haas, to describe their general purpose, polyester polymeric plasticizer.

Specific gravity— $25^{\circ} \text{ C.}/15^{\circ} \text{ C.}=1.08$ .

Viscosity poises— $25^{\circ} \text{ C.}/1=23$ .

Refractive index—N 25/0=1.466.

Average molecular weight—2200.

Acid number—2.0 (max.).

Saponification number—500.

In compounding Hycar 1411 was mixed with Paraplex G50 on a Hobart Mixer. The vinyl resin was added and the filler then was added slowly. The mass was transferred

to a Baker Perkins Mill and blended for 1 hour, during this time stearic acid and zinc oxide were added. Sulfur was added toward the end of the mixing time.

The sample was cured in a press for 10 minutes at 310° F. A combination of the above listed compounds can be employed as fillers as exemplified in Example 6, as follows:

## EXAMPLE 6

|                         |      |
|-------------------------|------|
| Vinyl resin             | 50   |
| Hycar 1411              | 43   |
| Hycar 1312              | 100  |
| Paraplex G50            | 50   |
| Dibutyl phthalate       | 35   |
| Zinc oxide              | 5    |
| Stearic acid            | 1    |
| Sulfur                  | 2    |
| Antimony oxide (filler) | 725  |
| Barium sulfate (filler) | 700  |
|                         | 7011 |

It has been found that by the addition of  $\text{BaSO}_4$  to other fillers a higher percentage of filler could be added. This is due to the low oil absorption of  $\text{BaSO}_4$ , thereby allowing more filler to be introduced into the formula. This is due to the fact that since  $\text{BaSO}_4$  has a very low oil absorption value, it does not absorb or utilize much of available plasticizer, thereby making available this plasticizer for other fillers. Thus, if other fillers with higher oil absorption value were used not as much plasticizer would be available. Another exceptional phenomena secured by employing  $\text{BaSO}_4$  as the filler is that it has been found that not much resinous binder is required to hold the  $\text{BaSO}_4$  particles together. What physical forces are influenced in this type of cohesive action is not understood.

Example 6 has other virtues than just affording a dense viscoelastic mass when cured. This formula possessing antimony oxide with vinyl chloride resin as a filler affords a self-extinguishing (core material). With the growing demand of fire retardancy in the building materials, this formula is excellent. This formula also offers an excellent acoustical caulking compound; which is an important part of an overall acoustical system. The formula can be easily molded with the fingers. This acoustical putty-like or acoustical caulk compound offers the acoustical field a highly specialized and needed acoustical caulk for acoustical installation applications.

Thus, the present invention produces a very high quality structure having very excellent sound transmission loss characteristics.

The embodiments of the invention in which an exclusive property or privilege is claimed are defined as follows:

1. A high density viscoelastic material having high sound transmission loss characteristics comprising the following elements and the following ratios by weight:

|                    |      |
|--------------------|------|
| Polyvinyl chloride | 400  |
| Plasticizers       | 410  |
| Kenflex            | 200  |
| Celluflex          | 20   |
| Barium sulfate     | 5200 |
|                    | 6230 |

wherein said plasticizer consists of:

|                       |     |
|-----------------------|-----|
| Tricresyl phosphate   | 170 |
| Diethyl phthalate     | 120 |
| Diiso-octyl phthalate | 120 |

wherein said Kenflex consists of synthetic polymer of aromatic hydrocarbons



avg. mol. wt. 662, melting point 160,

and wherein said Celluflex consists of alkyl epoxy stearate (4.5% oxirane oxygen).

2. A high density viscoelastic material having high sound transmission loss characteristics comprising the following elements and the following ratios by weight:

|    |                         |      |
|----|-------------------------|------|
| 5  | Powdered nitrile rubber | 200  |
|    | Polyvinyl chloride      | 150  |
|    | Plasticizer             | 200  |
|    | Stabilizer (vinyl)      | 5    |
| 10 | Barium sulfate          | 1500 |
|    |                         | 2055 |

3. A high density viscoelastic material having high sound transmission loss characteristics comprising the following elements and the following ratios by weight:

|    |                |        |
|----|----------------|--------|
| 15 | Natural rubber | 100    |
|    | Zinc oxide     | 5      |
|    | Stearic acid   | 2      |
| 20 | Amax           | 1      |
|    | Methyl zimate  | 0.25   |
|    | Su'fur         | 0.75   |
|    | Reogen         | 5      |
| 25 | Barium sulfate | 570    |
|    |                | 684.00 |

wherein said Amax consists of N-oxydiethylene benzothiazole-2-sulfenamide; and wherein said Reogen consists of mixture of oil soluble sulfonic acid of high molecular weight with a paraffin oil.

4. A high density viscoelastic material having high sound transmission loss characteristics comprising the following elements and the following ratios by weight:

|    |                         |     |
|----|-------------------------|-----|
| 35 | Vinyl resin             | 50  |
|    | Hycar 1411              | 43  |
|    | Hycar 1312              | 100 |
|    | Paraplex G50            | 45  |
| 40 | Stearic acid            | 1   |
|    | Zinc oxide              | 5   |
|    | Sulfur                  | 2   |
|    | Aluminum oxide (filler) | 700 |
|    |                         | 946 |

45 wherein said resin is a polyvinyl resin having a specific viscosity in the range from 0.5 to 0.53 and a specific gravity of 1.4 and wherein said Hycar 1411 is a copolymer of butadiene and acrylonitrile of high acrylonitrile content having a specific gravity of 1.0 and a viscosity of about 115; wherein said Hycar 1312 is a copolymer of butadiene and acrylonitrile with a specific gravity of about 0.98, and wherein said Paraplex G50 is a polymeric plasticizer having a specific gravity of about 1.08 and average molecular weight of about 2200 and a saponification number of about 500.

5. A high density viscoelastic material having high sound transmission loss characteristics comprising the following elements and the following ratios by weight:

|    |                         |      |
|----|-------------------------|------|
| 60 | Vinyl resin             | 50   |
|    | Hycar 1411              | 43   |
|    | Hycar 1312              | 100  |
|    | Paraplex G50            | 50   |
|    | Dibutyl phthalate       | 35   |
| 65 | Zinc oxide              | 5    |
|    | Stearic acid            | 1    |
|    | Sulfur                  | 2    |
|    | Antimony oxide (filler) | 725  |
|    | Barium sulfate (filler) | 700  |
|    |                         | 1711 |

wherein said Hycar 1411 is a copolymer of butadiene and acrylonitrile having a specific gravity of 1.0 and a viscosity of about 115, wherein Hycar 1312 is a copolymer of butadiene and acrylonitrile having a specific gravity

of about 0.98, and wherein said Paraplex G50 is a polyester plasticizer having a specific gravity of about 1.08, an average molecular weight of about 2200, and a saponification number of about 500.

6. A viscoelastic material as set forth in claim 1 <sup>5</sup> faced on at least one side with a stiff facing material.

7. A viscoelastic material as set forth in claim 2 faced on at least one side with a stiff facing material.

8. A viscoelastic material as set forth in claim 3 faced on at least one side with a stiff facing material.

9. A viscoelastic material as set forth in claim 4 faced on both sides with a facing panel.

10. A viscoelastic material as set forth in claim 5 faced on both sides with plywood panels.

|           |         |                      |        |
|-----------|---------|----------------------|--------|
| 3,056,707 | 10/1962 | Helbing et al. ----- | 181—33 |
| 3,087,566 | 4/1963  | Watters -----        | 181—33 |
| 3,253,947 | 5/1966  | McCluer et al. ----- | 181—33 |

## FOREIGN PATENTS

|         |         |                |
|---------|---------|----------------|
| 604,197 | 8/1960  | Canada.        |
| 810,661 | 10/1951 | Germany.       |
| 909,838 | 11/1962 | Great Britain. |

## OTHER REFERENCES

Akustische Beihefte, supplement published by Acustica (German periodical), Heft 1 (Supplement 1) of 1961, pp. 264-269.

15 ROBERT S. WARD, JR., *Primary Examiner.*

U.S. Cl. X.R.

156—281; 181—31

## References Cited

## UNITED STATES PATENTS

|           |         |                    |         |
|-----------|---------|--------------------|---------|
| 2,343,600 | 3/1944  | Weimann -----      | 156—281 |
| 2,391,489 | 12/1945 | Stamm et al. ----- | 156—281 |

UNITED STATES PATENT OFFICE  
CERTIFICATE OF CORRECTION

January 28, 1969

Patent No. 3,424,270

Seymour Hartman et al.

It is certified that error appears in the above identified patent and that said Letters Patent are hereby corrected as shown below:

Column 7, line 20, "7011" should read -- 1711 --. Column 9, line 9, "stifl" should read -- stiff --.

Signed and sealed this 17th day of March 1970.

(SEAL)

Attest:

Edward M. Fletcher, Jr.

Attesting Officer

WILLIAM E. SCHUYLER, JR.

Commissioner of Patents